

# UNITED STATES PATENT OFFICE.

URIAH BAKER, OF ELWOOD, NEW YORK.

## IMPROVEMENT IN ROOFING COMPOUNDS.

Specification forming part of Letters Patent No. **222,437**, dated December 9, 1879; application filed May 31, 1879.

*To all whom it may concern:*

Be it known that I, URIA BAKER, of Elwood, in the county of Suffolk and State of New York, have invented certain new and useful Improvements in Roofing Compounds; and I do hereby declare that the following is a full, clear, and exact description of the construction and operation of the same.

My invention relates to roofing composition; and it consists in compounding fire-clay, anthracite-coal ashes, fine sand, cement, lime, and linseed-oil in certain proportions, for the purpose of producing a compound of a proper consistency to be employed as a paint for roofs or other weather exposures, or of a consistency suitable for receiving and retaining sand or gravel, especially upon surfaces which are nearly flat, or having but the usual incline of flat roofs, or of proper consistency to be used for the purpose of cement.

I have discovered that the following proportions of the several ingredients form the best compound: First, fire-clay, thoroughly dried and pulverized, fifty parts; second, the ashes of anthracite coal, well sifted and in a fine state, twenty-five parts; third, fine sand, twelve parts; fourth, cement, ten parts; fifth, lime, water-slaked until reduced to a powder,

three parts; these parts to be thoroughly mixed together and ground in linseed-oil, either thick in its consistency for coating sand and gravel roofing, or thin for painting only, or thoroughly mixed together in linseed-oil without grinding, of a proper consistency to be used for the purpose of cement.

I am aware that coal-ashes have been treated and used in the formation of mineral paint, and I do not, therefore, broadly claim them; but

What I do claim is—

In a compound for a roofing-paint, coating, or cement, fifty parts of fire-clay, twenty-five parts of ashes of anthracite coal, twelve parts of fine sand, ten parts of cement, three parts of powdered slaked lime, all the parts thoroughly mixed and ground, or mixed and not ground, in linseed-oil, or their equivalents in kind or proportion, as and for the purposes substantially as set forth.

In testimony that I claim the above I have hereunto subscribed my name in the presence of two witnesses.

URIAH BAKER.

Witnesses:

HENRY C. BAKER,  
ISAAC H. BAKER.